

April 2, 1957

A. MURRAY ET AL

2,787,543

PHOTOGRAPHIC COLOR REPRODUCTION PROCESS

Filed Oct. 9, 1952



# United States Patent Office

2,787,543

Patented Apr. 2, 1957

1

2,787,543

## PHOTOGRAPHIC COLOR REPRODUCTION PROCESS

Alexander Murray and Earl M. Robertson, Rochester, N. Y., assignors to Eastman Kodak Company, Rochester, N. Y., a corporation of New Jersey

Application October 9, 1952, Serial No. 313,822

1 Claim. (Cl. 96—14)

This invention relates to a process in color photography and more particularly to a color process involving the superimposition of colored polymeric relief images.

In the early stages of color photography, colored reproductions were made by the subtractive method of color photography by superimposing suitably colored gelatin relief images. It was early recognized that the various superimposed images should not undergo dimensional change in the presence of heat and moisture and this led to the use of water-resistant supports for the superimposed elements as well as for the transfer sheet upon which the superimpositions were made. As early as 1891, collodion-coated paper was used for this purpose and present-day processes of this type still utilize sensitive tissues having a cellulose derivative or other similar moisture-resistant support. Glass and even wire screen have also been used to prevent the distortion of the images. In recent years in an effort to obtain films for superimposing which are more resistant to distortion in the presence of moisture, dichromate-sensitized colloid material such as dichromate-sensitized viscose and regenerated cellulose sheeting have been used. Obviously, such systems are relatively insensitive to light according to modern standards, are still moisture-sensitive, and are relatively unstable among other disadvantages.

In certain other well known processes of color photography in current use, the problem of distortion and registration of colored photographic images has been met by superimposing the layers recording the separate aspects of a colored subject as in multilayer color films. However, in certain instances such as in the printing trade when it is desired to obtain proofs of colored printing plates, the superimposition of individually colored elements is still desired.

We have discovered that if there are employed for the formation of suitably subtractively colored relief images certain solvent-soluble polymeric materials having relatively high light-sensitivity and which are relatively impermeable to moisture, the long-needed process yielding more dimensionally stable images for superimposition is made available and some disadvantages of prior art methods are overcome.

One object of our invention is, therefore, to provide suitable light-sensitive polymeric materials for use in making superimposed subtractively colored relief images. Another object is to provide a method for making the relatively dimensionally stable subtractively colored images for superimposition.

In the broadest phases of our invention we utilize a light-sensitive photographic element having a support preferably transparent and having high dimensional stability to some non-aqueous liquids, such as viscose, regenerated cellulose or a substantially fully esterified cellulose ester such as cellulose triacetate and particularly surface-hydrolyzed cellulose acetate. This support is coated with a layer of an organic solvent-soluble light-sensitive polymeric material having monomeric units containing groups of the structure



wherein  $n$  is 2 or 3 and  $\text{R}$  represents a mononuclear aromatic group of the benzene series or a polynuclear aromatic

2

group as of the naphthalene series. A typical polymer is a cinnamic acid ester of polyvinyl alcohol.

In the accompanying drawings are shown in greatly enlarged cross-sectional view in Figs. 1—4 the appearance of three representative sensitive elements at various stages in the process of our invention wherein are prepared cyan, magenta and yellow colored relief images on transparent supports which are superimposed to form a full colored reproduction.

Our invention will now be described with particular reference to the accompanying drawings.

### EXAMPLE 1

As shown in Fig. 1 of the drawings, three sensitive elements are provided having supports 10, 20 and 30, each carrying a layer of light-sensitive polymeric material 11, 21 and 31. A support suitable for this purpose is surface-hydrolyzed cellulose triacetate about .003 inch thick. Each of the three supports can be coated with a light-sensitive layer from a composition such as the following:

15 Anisalacetylpolystyrene ----- grams... 6  
Furfural ----- cc... 100  
Tricresyl phosphate ----- grams... 0.3

The polymer in the above composition is prepared as described in the Unruh et al. U. S. patent application Serial No. 246,516, filed September 13, 1951, now U. S. Patent 2,716,097, Example 3 thereof, by the condensation of anisaldehyde with polyvinyl acetophenone in the presence of mineral acid.

20 After drying the coated elements, they are exposed through the base separately by contact with the usual continuous tone subtractive primary color separation negatives at 4 feet from a 35-ampere carbon arc. With the particular set of negatives used, the magenta negative required 10 seconds' exposure, the cyan 7 seconds and the yellow 12 seconds, the exposure difference being due primarily to differences in maximum density of the separation negatives. The result of the exposure is to insolubilize the polymeric coating adjacent to the support in the region of the exposure.

25 30 The exposed elements are then developed in an organic solvent solution in order to remove the unexposed area. This development can be carried out with a mixture of 10 percent benzaldehyde in methyl ethyl ketone for 1½ minutes followed by rinsing in a fresh solution of the mixed solvents. The result is to obtain three elements as shown in Fig. 2 of the drawings, each carrying a relief image of solvent-insoluble anisalacetylpolystyrene resin in areas 12, 22 and 32 of the elements, corresponding to the highlights of the color separation negatives to which each had been exposed. The elements having supports 10, 20 and 30 now carry the respective resin relief images 12, 22 and 32 corresponding to the blue, green and red light aspects of the original subject respectively.

35 40 45 50 55 The relief images are now colored subtractively in a suitable manner by means of a solvent dye bath such as the following:

### Solvents (cc.) and dyes (gm.)

|    |                    | Magenta Bath A | Yellow Bath B | Cyan Bath C |
|----|--------------------|----------------|---------------|-------------|
| 60 | Xylene             | 96 or 50       | 50            | 50          |
|    | Furfural           | 4              | 4             | 50          |
|    | Benzaldehyde       | 2              | 2             | 2.5         |
| 65 | Dye A <sup>1</sup> |                |               | 1.7         |
|    | Dye B <sup>2</sup> |                |               |             |
|    | Dye C <sup>3</sup> |                |               |             |

<sup>1</sup> Azomethine dye from 2-cyanoacetylcoumarone coupled with 2-amino-5-diethylaminotoluene.

<sup>2</sup> Azomethine dye from  $\omega$ -benzoylacetanilide coupled with

<sup>3</sup> N,N-diethyl-p-phenylenediamine.

<sup>3</sup> Azomethine dye from 1-hydroxy-2-[ $\beta$ -(4'-acetamido)phenyl]naphthamide (Example 2, U. S. Patent 2,589,004) coupled with 2-amino-5-diethylaminotoluene.

As is apparent, baths A, B and C are used for dyeing the images 22, 12 and 32 respectively and following this step each element is rinsed in a suitable solvent in which the dye has little if any solubility, for example, n-hexanol following the magenta bath A, isopropanol following bath B and one of the xylenes following bath C.

The dyed elements now appear as shown in Fig. 3 of the drawings wherein the elements having supports 10, 20 and 30 are shown as carrying the yellow, magenta and cyan dyed reliefs 13, 23 and 33 respectively.

In case the three dyed relief images on their separate supports are to be utilized as proofs for color printing plates or for simply viewing as full color reproductions, they are superimposed as shown in Fig. 4 of the drawings, and viewed by transmitted light. If desirable, the elements may instead be superimposed on a white background for viewing by reflection. It will be apparent that since the coloring material in each of the relief images is locked into a moisture-impermeable resinous relief image, the dyes therein are appreciably more stable under adverse conditions of temperature and humidity known to gradually deteriorate dyes, than are dye images in prior moisture susceptible elements such as mentioned.

#### EXAMPLE 2

In a manner similar to Example 1, subtractively colored dye images are prepared on sheets of cellophane to effect coloring of at least the exposed regions of the elements before superimposition. In doing so, if the commercial product is used usually consisting of viscose coated with various substances, it is advisable in order to obtain utmost adherence of the relief images to the support, to remove any solvent-soluble coatings on the surface of the sheet with solvent such as a mixture of ethylene dichloride and ethyl acetate followed by a wash with methyl cellosolve acetate. Three such sheets are then coated with the following compositions:

|                         |       |     |
|-------------------------|-------|-----|
| Anisalacetylpolystyrene | grams | 10  |
| Furfural                | cc.   | 100 |
| Tricresyl phosphate     | grams | 1   |

After each sheet has been coated and dried, it is exposed through the base in contact with one of three continuous tone color separation negatives to a 35-ampere carbon arc at a distance of 4 feet for 1½ minutes. The exposed sheets are then developed in a tray of methyl ethyl ketone for 3 minutes followed by a rinse in the same solvent for 1½ minutes and a short rinse in methyl Cellosolve acetate. After this, each sheet is dyed in a solvent solution of the appropriate subtractively colored dye corresponding to the color separation aspect each represents, such as the following:

|                 |       |    |
|-----------------|-------|----|
| Dye             | grams | 2  |
| Xylene          | cc.   | 86 |
| n-Hexyl alcohol | cc.   | 10 |
| Benzaldehyde    | cc.   | 4  |

Suitable cyan, magenta and yellow dyes for use in this dye solution are yellow dyes such as the azo dye obtained by coupling o-nitro-p-chloroaniline with 5,5-dimethyl-1,3-cyclohexadione according to Example 4 and claim 7 of McNally et al. U. S. Patent 2,183,997, December 19, 1939; a magenta dye such as the azo dye obtained by coupling 2-chloro-4-nitroaniline with bis-(β-hydroxyethyl) aniline as described in Geigy Swiss Patent 169,946, June 15, 1934, and a blue or cyan colored dye such as the azo dye obtained by coupling 2-amino-3,5-dinitrobenzenesulfonethylamide with 1-β,γ-dihydroxy-propyl-2,7-dimethyltetrahydroquinoline as described in the Dickey et al. U. S. Patent 2,391,886, January 1, 1946.

After dyeing the relief images with the respective dye solutions they can be rinsed with n-hexyl alcohol, dried and superimposed in the desired manner to yield full color reproductions for viewing for the desired purposes mentioned previously.

Other transparent supports upon which the light-sensitive compositions may be coated and upon which the colored relief images may be formed are, for example, films of polyvinyl chloride, polyacrylonitrile, polyamides, phenolic resins and the like as will occur to those skilled in the art.

#### EXAMPLE 3

The dyed polymeric relief images can more advantageously be formed from predyed light-sensitive polymeric compositions such as the following:

|                                         |       |     |
|-----------------------------------------|-------|-----|
| Dye                                     | grams | 1   |
| Polyvinyl cinnamate                     | do    | 10  |
| Furfural                                | cc.   | 100 |
| 4,4'-Tetramethyldiamino-diphenyl ketone | grams | 1   |

The dyes particularly suitable for use in the dye solutions above for dyeing the polymeric materials are the "spirit-soluble" dyes as opposed to oil-soluble or water-soluble dyes, or mixtures of dyes, such as

|                      | C. I. No. |
|----------------------|-----------|
| Chrysoidine          | 20        |
| Chrysoidine 3R       | 21        |
| Bismark Brown R      | 332       |
| 25 Malachite Green   | 657       |
| Para Rosaniline Base | 676       |
| Fuchsine H Base      | 677       |
| Methyl Violet Base   | 680       |
| Spirit Blue B        | 689       |
| 30 Victoria Blue B   | 729       |
| Induline Base B      | 860       |

Reference can be made to the "Technical Manual and Yearbook of the American Association of Chemists and Colorists," 1951, for the "spirit-soluble" dyes.

A further group of "spirit-soluble" dyes valuable for this purpose are basic dyes, especially tannin lakes of basic dyes, of which the following are representative.

|                           |
|---------------------------|
| Rotalin Blué B            |
| Rotalin Yellow G Supra    |
| Rotalin Green Y           |
| Rotalin Red               |
| Rotalin Brilliant Blue 2B |
| Rotalin Violet            |
| Rotalin Black RM          |

The first three dyes enumerated are respectively substantially identical to tannin lakes of Victoria Blue B, Auramine O (C. I. 655), Victoria Green (C. I. 657). Rotalin Red corresponds to a mixture of Rhodamine 6 SDN (C. I. 752) and Auramine O (C. I. 655), the remaining dyes also being tannin lakes.

It is therefore apparent that basic dyes per se and particularly tannin and similar lakes thereof are especially useful for dyeing the light-sensitive coating compositions.

Another group of "spirit-soluble" dyes of equal value in this process are salts of acid dyes such as the following:

|                     |
|---------------------|
| Luxol Fast Black PS |
| Luxol Fast Blue MBS |
| Luxol Fast Red BB   |
| Luxol Fast Yellow T |

These dyes are arylguanidine salts of acid dyes.

These dyes, particularly the Rotalin dyes, are preferred since they are not appreciably soluble in the solvent developers used for developing the polymeric relief images such as trichloroethylene or 20% methyl Cellosolve acetate in xylene.

The dye compositions are coated for example on sheets of surface-hydrolyzed cellulose acetate, gelatin, subbed cellulose esters or on polyvinyl chloride. The sheets are then exposed to continuous toned negatives as above mentioned by exposure through the support, for example, the magenta-colored sheet receiving 1¼ minutes' exposure,

the cyan 1½ minutes and the yellow 2 minutes at 4 feet from a 35-ampere carbon arc, when employing the Luxol dyes. Different exposure times up to 5 minutes are required depending upon the dyes used. The exposed films are then developed with solvent vapor such as trichloroethylene for about 20 seconds or in a tray of solvent such as 20% methyl Cellosolve acetate in xylene for up to 5 minutes to remove the dyed polymer in the areas not insolubilized by exposure to the continuous tone negative. When the three single colored transparencies are superimposed, a full color transparency of good quality is obtained.

#### EXAMPLE 4

When it is desired to obtain a black-and-white monochrome relief image or to add a fourth color to a 3-color print or transparency in the form of a black resin image, suitable images are prepared by coating a black light-sensitive composition such as the following on to a suitable support such as surface hydrolyzed cellulose acetate.

|                                        |       |      |
|----------------------------------------|-------|------|
| Polyvinyl cinnamate                    | grams | 7.5  |
| Furfural                               | cc    | 70   |
| Xylene                                 | cc    | 30   |
| Black dye                              | grams | 0.75 |
| 4,4'-tetramethyldiaminodiphenyl ketone | do    | 0.75 |

A suitable black dye for this composition is a "spirit-soluble" dye such as Spirit Nigrosine (C. I. 864). As previously mentioned, dyes of this type are especially suitable since they are retained by the polymeric relief images during the development step. As in the previous examples, the sensitive coating is exposed through the base in contact with a continuous tone photographic negative for 2 to 5 minutes at a distance of 4 feet from a 35-ampere carbon arc. The image is developed for 2½ minutes in a 10 percent solution of furfural in xylene or for up to 5 minutes in the tray developer of Example 3 and rinsed for 30 seconds in a fresh mixture of the same solvents. The dye is insoluble in this developing solution and therefore does not bleed out into the solvents. There results a clean, black, continuous tone image reproducing a density scale of approximately 1.5 in the negative. In an alternative method, the relief image is developed by immersing the exposed sheet in vapor of trichloroethylene. The unexposed portion of the polymer dissolves in the condensate carrying the dye with it physically while the dye insoluble in the trichloroethylene is retained by the insoluble exposed polymer to produce a neutral continuous tone transparent positive image.

#### EXAMPLE 5

Our process can be applied particularly to proofing color printing plates as follows: on three separate sheets of surface-hydrolyzed cellulose acetate, coatings are made with three predyed polyvinyl cinnamate solutions of the same composition as given in Example 3 above. Each sheet is then exposed for from 1½ to 8 minutes (depending on the dye used) at 4 feet from a 35-ampere carbon arc through a 266-line (or other appropriate ruling) halftone color separation negative corresponding to the color of the coating in vacuum contact with the surface of the polymer. The exposed sheets are then developed separately in a tray of 10 percent furfural in xylene for 2 minutes or in 20% methyl Cellosolve acetate in xylene for up to 5 minutes and rinsed for about 30 seconds in fresh solvent mixture. After drying the solvents from the polymeric reliefs, they are superimposed to produce a tricolor halftone color proof. With the proper selection of dyes, dye concentration, and exposure, reproducible color proofs can be made which accurately predict the outcome of the final press sheet.

From the above description it will be apparent that since the light-sensitive polymeric materials are highly stable, colorless or precolored light-sensitive polymeric coated sheets in different colors can be supplied to the

trade for quickly making color proofs. Such products conveniently include stripping films having temporary supports from which the solvent developed colored relief images on thin transparent supports can be stripped for superimposing to form a full color reproduction. Also the relatively high light-sensitivity of the polymeric materials used in our invention promises extensive commercial utility for the light-sensitive products for exposure directly in a camera for the production of continuous and halftone multicolor images. The prior art processes for making colored reproductions by superimposing colored relief images obviously suffered in part due to the low speed of the polymeric materials used as well as the poor resistance of such materials to moisture.

15 In large scale production, for example, involving mechanical methods for laminating the above individually colored transparencies together, our process provides an intrinsically cheaper method than obtaining color reproductions by means of integral tripack color transparencies based upon silver halides and color development methods. Thus, while the particular source of the color separation aspects used in exposing the light-sensitive polymer coatings is not critical, negatives, for example, obtained by exposure of well known three-layer stripping films having differently sensitized silver halide emulsions, or negatives exposed in three-color one-shot cameras, are well suited for use in our process:

20 The light-sensitive polymers given for illustration in the above examples are by no means exhaustive of those contemplated for use in our invention. Other polymers represented by that of Example 1, the preparation of which are disclosed in the mentioned Unruh et al. invention and in the Unruh et al. U. S. patent application Serial No. 246,517, filed September 13, 1951, now U. S. 25 Patent 2,706,725, granted May 19, 1955, are the organic solvent-soluble light-sensitive materials containing polymeric units having the group



in which R is a mononuclear or a polynuclear aromatic group particularly of the benzene and naphthalene series in which the nuclei are substituted or not, particularly the polymers made by substantially completely acetylating a styrene polymer and condensing with an aromatic aldehyde, or a vinyl acetophenone polymer condensed with an aromatic aldehyde. These polymers contain monomeric units having the general structure



in which n is a number from 1 to 4 and Q is a mononuclear or polynuclear aromatic group particularly of the benzene or naphthalene series substituted or not and D is a single bond or aryl group of the benzene or naphthalene series. Accordingly, other polymers useful in our invention contain combined polymeric units of the following:

- Isopropylbenzal acetylstyrene
  - 65 p-Hydroxybenzal acetylstyrene
  - p-Dimethylamino acetylstyrene
  - o-Chlorobenzal acetylstyrene
  - p-Acetamidobenzal acetylstyrene
  - p-Sulfonylbenzal acetylstyrene
  - 70 Anisal acetylstyrene
  - Veratral acetylstyrene
  - Anisal acetyl-o-methoxystyrene
  - p-Hydroxybenzal acetyl-o-methoxystyrene
  - o-Chlorobenzal acetyl-o-chlorostyrene
  - p-Chlorobenzal acetyl-2,5-dimethylstyrene
- 75

Anisal acetyl-p-phenoxy styrene  
 Anisal acetyl-p-bromostyrene  
 Toluol acetyl-3,4-dimethoxystyrene  
 Anisal acetyl-o-fluorostyrene  
 $\alpha$ -naphthal acetylstyrene  
 Anisal benzal-acetylstyrene  
 Anisalvinylmethyl ketone  
 Benzal acetylestyrene  
 Benzal acetyl-o-methoxystyrene  
 Benzal acetyl-o, m-, p-chlorostyrenes  
 Benzal acetyl-o, m-, p-bromostyrenes  
 Benzal acetyl-p-benzylstyrene  
 Benzal acetyl-p-phenoxy styrene  
 Benzal acetyl-3,4-dichlorostyrene  
 Benzal acetyl-2,5-dimethylstyrene  
 Benzal acetyl-m-methylstyrene  
 Benzal acetyl-m-tert. butylstyrene  
 Benzal acetyl-3,4-dihydroxystyrene

The preferred light-sensitive materials are polymers of vinylacetophenones condensed with a suitable aromatic aldehyde such as anisaldehyde.

Other suitable light-sensitive polymers are the cinnamal vinylacetophenone polymers disclosed by the Unruh et al. application Serial No. 246,515, filed September 13, 1951, now U. S. Patent 2,716,102. These polymers contain monomeric units having the general formula



wherein D represents a single bond or a mononuclear arylene group, Q represents a mononuclear aryl group, n represents a whole number from 1 to 4, and R is alkyl, preferably of 1 to 4 carbon atoms, and are obtained by condensing a cinnamic aldehyde with, for example, a polymer of a vinyl acetophenone compound; for example:

Polycinnamalacetylstyrene  
 Poly- $\alpha$ -n-amylocinnamalacetylstyrene  
 Poly-p-chlorocinnamalacetylstyrene  
 Poly-m-nitrocinnamalacetylstyrene  
 Poly-o-chlorocinnamalacetylstyrene  
 Poly-p-methoxy cinnamalacetylstyrene  
 Poly-p-methylcinnamalacetylstyrene  
 Poly-p-chlorocinnamalacetyl-o-methoxystyrene  
 Poly-p-methylcinnamalacetyl-o-chlorostyrene  
 Polybenzalcinnamalacetylstyrene  
 Polycinnamalmethylvinylketone

The polymeric material polyvinyl cinnamate used in Example 4 was prepared by the methods of the Minsk et al. U. S. patent application Serial No. 207,052, filed January 20, 1951, and is the substantially fully acylated cinnamic acid ester of polyvinyl alcohol. While the substantially fully esterified cinnamic acid esters of polyvinyl alcohol defined in the Minsk et al. invention are preferred for use in our invention since they are least moisture-susceptible, those cinnamic acid esters containing at least 60 mole percent of any cinnamoyl ester groups are useful in our invention in the predyed or colorless light-sensitive elements of the foregoing examples. Cinnamic acid esters of other materials such as of starch and hydroxy alkylated cellulose (Minsk et al. U. S. patent application Serial No. 308,284, filed September 6, 1952, now abandoned) can also be used to good advantage. It will also be apparent that we can use in the light-sensitive elements, mixtures of two or more of the light-sensitive polymers and each of the three or more elements used in making full-color reproductions may comprise a different light-sensitive polymer. As will also be appa-

rent to those skilled in the art, useful results can be obtained when the three light-sensitive polymeric elements are suitably sensitized and are exposed through suitable filters directly to the colored scene or subject to be reproduced, for example, by use of tricolor filter exposures in a camera to obtain line, halftone or continuous tone reproductions. Optical sensitization of the compositions is aided by use of the thiazole sensitizers disclosed in the West and Robertson U. S. patent application Serial No. 314,806, filed October 15, 1952 now U. S. Patent 2,732,301.

In Examples 3 and 4 are illustrated the use of sensitizing agents for the polymeric materials, for example, 4,4'-tetramethyldiaminodiphenyl ketone. Other sensitizing agents useful in conjunction with any of the above enumerated sensitive polymers are the nitro, triphenylmethane, anthrone, quinone, diphenylketone and thiazole sensitizers respectively of the Minsk et al. U. S. patent application Serial No. 148,684, filed March 9, 1950, now U. S. Patent 2,610,120, granted November 7, 1950, the Minsk et al. U. S. patent application Serial Nos. 207,048-51, filed January 20, 1951, now U. S. Patents 2,690,966, 2,670,285-7, and the above West et al. invention. Typical sensitizing agents of those inventions are 2,4,6-trinitroaniline, Crystal Violet dye, 2-keto-3-methyl-1,3-diazabenzanthrone and 1,2-benzanthraquinone. The preferred sensitizing agent for all of the above uses where sensitizers are desired is 2-benzoylmethylene-1-methyl- $\beta$ -naphthothiazoline because of its superior sensitizing activity and stability in combination with the polymer coatings.

From the above description it will be apparent that we have provided means for preparing colored relief images on transparent supports for superimposing. Our invention is further adapted to preparing such colored polymeric relief or resist images upon metallic supports such as are useful in the printing trade. That is, in the preparation of resists upon metal plates in photoengraving and photolithography it is desirable to provide a means for visual examination of the resist image before etching or proofing the plate. Consequently, when using the light-sensitive organic solvent soluble polymers such as indicated above for forming resist images, it is desirable to either bathe the resist in dye solution or to incorporate coloring material into the light-sensitive polymer composition before formation of the resist image. The latter procedure is preferred partly since the after-dyeing step can be dispensed with. However, prior to our invention dyes have not been found which would not bleed from the resist images during the course of the solvent development step such as employed in Example 3. Now by use of the dyes, such as given above, in the initial light-sensitive polymer compositions a variety of solvents such as those given in Example 3 can be utilized for solvent development of a resist image on various metal plates. Accordingly, in the preparation of a zinc lithographic plate a composition such as set forth in Example 3 can be coated on a freshly counter-etched zinc plate, exposed to a suitable line or half-tone subject and developed in a solvent such as trichloroethylene in liquid or vapor form to obtain a well defined colored resist on the zinc surface. In a similar manner the other light-sensitive polymers can be sensitized with the indicated sensitizing agents, and resists formed on zinc, magnesium or other metal plates. In a similar manner colored polymeric images can be formed on other surfaces such as ceramic ware, glass, paper, plastic, etc. for purely decorative purposes.

What we claim is:

A method for preparing a colored photographic reproduction which comprises exposing to separate color aspects of a subject at least two photographic elements each carrying on a transparent support a layer of a light-sensitive organic solvent-soluble polyvinyl cinnamate subtractively colored with a spirit soluble dye, to insolubilize

the exposed areas of the layer, removing only the soluble areas of the exposed layers with an organic solvent in which said dye is insoluble to obtain subtractively colored relief images of insoluble polymer on each support corresponding to said color aspects, and superimposing the 5 resulting elements.

## References Cited in the file of this patent

## UNITED STATES PATENTS

|           |              |       |               |
|-----------|--------------|-------|---------------|
| 1,953,175 | Hebbel       | ----- | Apr. 3, 1934  |
| 2,577,984 | Warnecke     | ----- | Dec. 11, 1951 |
| 2,610,120 | Minsk et al. | ----- | Sept. 9, 1952 |

## FOREIGN PATENTS

|         |               |       |              |
|---------|---------------|-------|--------------|
| 384,364 | Great Britain | ----- | Dec. 8, 1932 |
|---------|---------------|-------|--------------|